

Dec. 27, 1949

H. B. SLOAN

2,492,666

HYDROGEN-FILLED THYRATRON

Filed March 15, 1946



INVENTOR  
Howard B. Sloan

BY  
Laurence Bunn  
ATTORNEY

Fig. 1

## UNITED STATES PATENT OFFICE

2,492,666

## HYDROGEN-FILLED THYRATRON

Howard B. Sloan, Swampscott, Mass., assignor to  
 Sylvania Electric Products Inc., Salem, Mass.,  
 a corporation of Massachusetts

Application March 15, 1946, Serial No. 654,564

7 Claims. (Cl. 250—27.5)

1

This invention relates to electron tubes such as thyratrons and particularly to hydrogen-filled thyratrons. The invention is especially applicable to tubes for producing short, sharp pulses, such as shown in my co-pending application Serial No. 585,491 filed March 29, 1945.

To increase the electron emission of such tubes, the base material, usually nickel, of the cathode should be extremely pure, much purer than any commercially available in the past. In addition, I have found that the addition of zinc to the tube is necessary to secure a low voltage drop, although the exact function of the zinc is not fully understood. The zinc may be added to the tube in any convenient manner, and some will generally remain on the glass of the tube unless driven off, but some of the zinc must be condensed on the part of the tube to secure the desired results. In one case, for example, where all the zinc was condensed on the glass, the voltage drop was 157 volts; when the zinc was driven back onto the electrodes of the tube by vaporizing it from the glass wall, the voltage dropped to 88 volts, about half its former value.

Other objects, features and advantages of the invention will be apparent from the following specification taken in conjunction with the accompanying drawings, in which:

Figure 1 is a vertical cross section of a tube according to the invention; and

Figure 2 is a perspective view, partly in section, of an alternative construction for the top of the tube.

In the figures, the glass tube 1 has the lead-in wire 2 sealed through and closing one of its ends with the stem 3 through which additional lead-in wires 4, 5 and 6 extend, sealed to and closing the opposite end. The tungsten filament coil 7 is attached at one end to the conductor 8 which supports it from the lead-in wire 5 to which it is electrically connected. A coating of refractory insulating material such as aluminum oxide is used on the filament turns to prevent short-circuiting thereof on sagging. The other end of filament coil 7 is connected by the metal tabs 9 and 10 to the disc 11 whose flanged edges 12 are attached to nickel cylinder 13, which is coated on its outside diameter with an electron emitting mixture of barium and strontium oxides. This coating is best terminated a short distance from each end of the cylinder. The bottom of the cylinder is attached by the disc 14 through which the conductor 8 passes and from which it is spaced or insulated. A disc of larger diameter 15 is attached to the disc 14 and extends beyond the

5 diameter of the cathode cylinder 13, to support the cathode shields 16 and 17 which may be attached to the flange or rim 18 at the outside of the disc. The two cathode shields are preferably spaced apart a short distance. The collar 19 supported from the top of shield 17 in turn supports the shielding discs 20, 21 and 22 which are spaced from each other and attached to the collar 19 by the conductors 23 and 24. The cathode 10 shields 16 and 17 may be supported by the wires extending from a collar 27 around the base of stem 3, to insure rigidity.

Anode 28 is a circular metal disc attached to and supported by the lead-in wire 2 over which 15 the glass bead 29 extends from seal 30 to a point close enough to the anode 28 to prevent flash over. The glass tube 31 concentric with the bead and spaced therefrom, extends along the entire length of the bead and merges with the bead into 20 the seal 30 through which the lead-in wire 2 extends to be attached to the contact 32 by the solder 33. A collar 34 around the free end of glass tube 31 is attached to the transverse disc 35 which shields the top of the anode 28. The grid 36 25 of metal gauze is attached to the flange edge 37 of disc 35 at the top of anode 28 and to the collar 38 below anode 28 from collar 38. The perforated disc or grid 39 is affixed to collar 38. The additional collar 40 connects the disc shield 41 to the 30 grid 39 and spaces it therefrom. The anode 28 is thus completely surrounded by a structure comprising the grids 36 and 39 through which electrons from the cathode 13 must pass to reach said anode 28. The spacing between the anode 28 and the various parts of the grid should be small 35 enough to prevent flash back between the parts. The shielding disc 41 serves to prevent any metal evaporated from the filament from depositing on the grid 39 and causing it to emit electrons. For the most part however, the material evaporated 40 from the cathode 13 will be deposited on the shield 41 concentric with the cathode.

The bottom part of the grid 36 is attached to 45 the metal cylinder 42 which helps to support it and also acts as an addition head shield for the cathode 13. Cylinder 42 is supported at its bottom by the wires 43 and 44 which are sealed into stem 3. The conducting ribbons 45 and 46 connect lead-in wires 43 and 44 with the cylinder 50 42 to insure good electrical contacts therewith. Tabs such as 47 may be used to assist in connecting lead-in wires 43 and 44 to the cylinder 42. The base 49 may be cemented to the bottom part of the tube 1 by the cement 50 and the lead-in wires 4, 5 and 6 may be connected to the contact prongs

51, 52, 53, 54 of the base which are insulated from each other. Prong 52 may be connected inside the base to prong 51 by the jumper connection 55.

The tube is of course, evacuated and filled with hydrogen at a pressure of  $\frac{1}{2}$  mm.

In operation current is passed through the filament 7 which serves to heat the nickel cylinder 13 and the emitting coating upon it. The electrons emitted therefrom pass through the gas in the tube and eventually through the grids 36 and 39 to reach the anode 28. The grids 36 and 39 can thus be used to control the starting of the discharge as in the usual thyratrons and because of the use of hydrogen as the gas filling the discharge will deionize rapidly when the anode voltage is removed.

Prior to my invention the clean up of hydrogen in tubes of this sort was a serious problem. I find that in a tube of my novel construction however, the hydrogen is not cleaned up appreciably. This appears to be due to the fact that the electrons are all emitted from the outside of the cylinder 13 and passed through the confined space between the cylinder and the shield. Barium or strontium particles sputtered from the cathode will be picked up by the inside surface of the shield 16. The combination of these barium and strontium particles with the hydrogen to form a hydride may be the cause of the hydrogen clean up and in my particular construction the particles fall on the shield close to the cathode, apparently under such equilibrium conditions as cause the hydrogen to be removed therefrom. The absence of cathode coating from the top 12 of the cathode insures that all the sputtered particles will come from the sides of the cathode. In tubes prior to my invention the sputtered particles appear to have had a comparatively free path through the interior of the tube.

I find also that it is well to operate the tube at currents in excess of the normal thermionic electron emission of the cathode for the temperature at which it is operated. For example, the cylinder 13 may have a diameter of  $\frac{1}{4}$  inch and a height of  $1\frac{1}{4}$  inches, with an uncoated space of 0.4 mm. at each end of the cylinder. This gives a coated area of about  $14 \text{ cm}^2$ , for the barium and strontium oxide coating; and yet peak currents as high as 350 amperes may be safely carried by the tube without reducing its life below the present rating of 500 hours. Actually I have found a coating area extending from a point 0.4 cm. from the top of the cylinder 13 for a distance of 0.8 cm. downward to be sufficient for such a life.

The anode 28 and its surrounding grid structures 35-36-38 are spaced quite closely together, for example, 0.80 inch, and will not flash over with the gas pressure used, because of the well known short-path principle. However, were it not for the bead 29, flash over could occur between the grid structure 35, 36, 39 and the more remote parts of the lead-in wire 2 inside the tube. The beading prevents this flash over and should extend close enough to the anode 29 to insure a short enough path to the unbeaded portion of the lead-in tube to prevent flash over. The space tube 31 is an additional safeguard and also helps to support the disc 35. For example, my tube may use an anode voltage as high as 16,000 volts without flash over under those conditions. The distance from the anode 28 to the outer edge 56 of the seal 30 should be quite long to prevent electrolysis at the seal. For the voltage used, I find a distance of about 7.2 cm. to be sufficient.

The distance inside the tube from the anode 28 to the inner edge 59 of the seal is more important, and should be about 5.3 cm. for the voltage used.

The tube may be made somewhat shorter by making the seal in a reentrant form as shown in Figure 2. In this case the tube 58 extends into the enclosing envelope and outward again as tube 31 to be sealed to the bead 29 at point 59, which then extends upward out of the tube. The grid support collar 34 is then attached to the reentrant tube 58 as shown.

The oxides in the coating on cathode 13 may, of course, be applied as carbonates and converted to the oxides by heating during exhaust in the manner well-known to the art.

When not carrying current the voltage drop across the tube may be 16,000 volts, but when application of sufficient voltage to the grid 36 causes the tube to "fire" and pass current, the voltage across the tube may be as low as 88 volts or less for a current of 300 amperes, the remaining voltage appearing in the load circuit. The grid voltage for "firing" the tube may be about 150 volts in some cases, although it is generally applied in such transient form as to make its measurement difficult.

The voltages and current here given are for the peak value of the pulse through the tube, as far as they can be ascertained. The average current through the tube may be less than an ampere.

The zinc 60 is shown on the glass envelope 1 in the drawing, but some of it will be present on the electrodes of the tube. In some cases a sufficient trace of zinc may adhere to the parts if some zinc vapor is present in the furnace in which the electrode parts are fired in hydrogen, for cleansing prior to insertion in the tube, although I prefer to add some zinc oxide—on the outside of skirt—when the tube is being assembled.

When the tube is being exhausted, hydrogen at 1 or 2 mm. of mercury pressure may be passed through the tube and the oxide heated, for example by high frequency induction, whereupon the oxide will be reduced to metallic zinc and vaporized onto the tube parts. When the tube elements are further heated during the usual exhaust procedure known to the art, the zinc will condense on the glass at the top of the tube, as shown at 60 in the drawing. After the bulb is finished and sealed, the zinc may be driven off the top of the tube and onto the tube elements by heating, in a flame, the glass when the zinc has deposited. As previously stated, this will reduce the tube voltage drop as much as half, in one particular case from 157 to 88 volts.

What I claim is:

1. An electron tube comprising a sealed envelope, a filling of hydrogen therein, electrodes therein, and zinc on said electrodes.

2. An electron tube having a sealed envelope containing hydrogen at low pressure, and a plurality of electrodes enclosed within said envelope, said electrodes including an anode, a thermionic cathode, and a grid interposed between and enclosing said anode and said cathode, said cathode having an oxide coating and having a surface trace of zinc.

3. An electron tube having an envelope containing hydrogen, and plural electrodes including a thermionic cathode, an anode, and a control electrode interposed between the cathode and the anode, said electrodes having a surface trace of zinc.

4. A thyratron including an envelope having

a hydrogen fill and enclosing a small quantity of zinc.

5. An electron tube comprising a sealed envelope, a filling of hydrogen therein at a low pressure of the order of 0.5 mm., an anode, a grid, and an oxide-coated cathode therein, and zinc on the surface of said anode, grid and cathode.

6. A thyratron having a sealed envelope, a filling of hydrogen therein at low pressure of the order of 0.5 millimeter, and electrodes therein including an anode, a grid and an oxide-coated cathode, said cathode having a base material of pure nickel, said electrodes having a surface trace of zinc.

7. An electron tube having a sealed envelope 15 containing hydrogen at low pressure, and a plurality of electrodes enclosed within said envelope, said electrodes including an anode, a thermionic

5

cathode and a grid interposed between said anode and said cathode, said cathode having a base material of pure nickel, an oxide coating on said base material, and a surface trace of zinc.

HOWARD B. SLOAN.

#### REFERENCES CITED

The following references are of record in the file of this patent:

#### UNITED STATES PATENTS

| Number    | Name         | Date          |
|-----------|--------------|---------------|
| 1,172,568 | Schroter     | Feb. 22, 1916 |
| 1,699,112 | MacRae       | Jan. 15, 1929 |
| 2,089,325 | Aldington    | Aug. 10, 1937 |
| 2,096,862 | Spencer      | Oct. 26, 1937 |
| 2,399,003 | Crapuchettes | Apr. 23, 1946 |